

[54] HIGH CURRENT DENSITY BRINE ELECTROLYSIS

[75] Inventors: James M. Kolb, Mentor; Charles R. Franks, North Madison; Barry A. Schenker, Mayfield Heights, all of Ohio

[73] Assignee: Diamond Shamrock Corporation, Cleveland, Ohio

[22] Filed: Apr. 19, 1973

[21] Appl. No.: 352,418

[52] U.S. Cl. .... 204/99, 204/128, 204/290 F

[51] Int. Cl. .... C01d 1/06, B23p 3/00, C01b 7/06

[58] Field of Search ..... 204/99, 128, 290 F

[56] References Cited

UNITED STATES PATENTS

3,701,724 10/1972 Entwistle et al. .... 204/290 F

3,671,415 6/1972 King et al. .... 204/290 F

|           |         |                       |           |
|-----------|---------|-----------------------|-----------|
| 3,663,280 | 5/1972  | Lee.....              | 204/290 F |
| 3,627,669 | 12/1971 | Entwistle et al. .... | 204/290 F |
| 3,491,014 | 1/1970  | Bianchi et al. ....   | 204/240 F |

Primary Examiner—G. L. Kaplan

Assistant Examiner—R. L. Andrews

Attorney, Agent, or Firm—Timothy E. Tinkler

[57] ABSTRACT

Described is a method of electrolyzing brine in a mercury cell, at applied current densities of at least 6 amperes per square inch, employing as the anode a titanium substrate bearing on at least a portion of the surface thereof a mixed oxide coating of from 30 to 90 percent stannic oxide, from 1.0 to 10 percent antimony oxide, from 1.0 to 50 percent of at least one platinum group metal oxide, and from 0.5 to 30 percent of a valve metal oxide selected from the group consisting of titanium and tantalum oxides.

5 Claims, No Drawings

## HIGH CURRENT DENSITY BRINE ELECTROLYSIS

## BACKGROUND OF THE INVENTION

The electrolysis of aqueous sodium chloride solutions, i.e., brine, in electrolytic cells employing a flowing mercury cathode is widely practiced. Basically, the process comprises passing a direct current between essentially parallel anodes and cathodes through the brine, thereby liberating chlorine at the anode and depositing sodium on the mercury as an amalgam.

The apparatus employed for this purpose is quite expensive and a primary concern in commercial operation is to obtain the maximum amount of production per unit of floor space. One method of so doing is to increase the anode current density at which the cell operates. However, with the graphite anodes originally employed, the maximum current density that could be employed without drastically reducing the useful life of the anode was on the order of 5.0 asi. Even with the advent of dimensionally stable anodes, e.g., platinum-coated titanium, while operation at higher current densities was at least theoretically possible it was soon found in practice that these anodes rapidly passivated, that is, the operating voltage exceeded that at which practical operation was possible. The apparent cause of this passivation was brine depletion across the cell, oxygen evolution increasing with decreasing brine concentration.

## STATEMENT OF THE INVENTION

Therefore, it is an object of the present invention to provide a method for electrolyzing brine in a mercury cell at high current densities.

It is a further object of the present invention to provide a method for the high current density operation of mercury type cells for the electrolysis of brine wherein a low anode wear-rate and an extended anode life may be achieved.

These and other objects of the present invention will become apparent to those skilled in the art from the specification and claims that follow.

It has now been found that, in a process for the electrolysis of brine in a cell employing a flowing mercury cathode, an improvement consists essentially of employing as the anode a titanium substrate bearing on at least a portion of the surface thereof a mixed oxide coating of from 30 to 90 percent by weight stannic oxide, from 1.0 to 10 percent antimony oxide, calculated as  $Sb_2O_3$ , from 1.0 to 50 percent of at least one platinum group metal oxide, and from 0.5 to 30 percent of a valve metal oxide selected from the group consisting of titanium and tantalum oxides, with the proviso that the mole ratio of tin to antimony oxides be between 85:15 and 95:5, and applying current to said anode at a rate of at least 6 amperes per square inch.

The foregoing improvement is particularly effective in the instance where the valve metal oxide is  $TiO_2$  and the "platinum group metal oxide" is a combination of  $RuO_2$  and  $IrO_2$ .

## DESCRIPTION OF THE PREFERRED EMBODIMENTS

The mercury cells to which the practice of the present invention may be applied may be of the horizontal, vertical, or inclined plane type, all of which are well known to those skilled in the art. Such cells and their operation are described, for example, at Kirk-Othmer,

Encyclopedia of Chemical Technology, Vol. 1, pages 688-695 (2nd Edition, 1963).

Typically such cells operate on aqueous sodium chloride solutions having concentrations at or approaching saturation (brine), e.g., 325 grams per liter, although sea water has been successfully electrolyzed in some instances. The distance between the parallel anodes and mercury cathode of the cell is kept quite low, often on the order of 0.1 to 0.3 inch. Such cells are operated at temperatures up to the boiling point of brine and at sodium-mercury amalgam concentrations on the order of from 0.1 to 0.15 percent, the latter factor being controllable to some extent by regulating the mercury flow rate. Conventional operation is at anode current densities on the order of 3 to 4 asi and up to 6 asi.

According to the present invention, the amount of current supplied to the cell is at least 6 amperes per square inch of anode surface, preferably 6 to 10 asi. At such increased current densities, the brine becomes severely depleted during its passage from inlet to outlet thereby increasing the amount of oxygen evolved at the anode surface and normally contributing to the rapid passivation of same.

However, this tendency toward passivation is greatly reduced when the anode comprises a titanium substrate bearing on at least a portion of the surface thereof a mixed coating of the oxides of tin, antimony, at least one platinum group metal, and a valve metal selected from the group titanium and tantalum. Such anodes also exhibit a long "life," i.e., a low platinum group metal wear-rate per ton of chlorine.

The conductive substrate is generally titanium, although a more conductive material, such as copper or aluminum, bearing a surface of titanium may be employed. Additionally, layers on the substrate intermediate the titanium and the coating, such as those described in U.S. Pat. No. 3,711,397, are contemplated. The configuration of the substrate may vary considerably but it is generally in the form of a sheet, particularly a foraminous sheet, such as expanded mesh.

What may be considered the first of the components in the coating composition is stannic oxide, preferably present in the form of crystalline  $SnO_2$  and employed within the range of from 30 to 90, especially 30 to 50, percent by weight of the total coating composition.

The antimony oxide component enters into the tin oxide crystal lattice, rendering same more electrically conductive. Although the antimony is present in an indeterminate oxide form owing to its entrance into the stannic oxide crystal lattice, it is expressed for convenience sake as  $Sb_2O_3$ . Thus, on this basis, the antimony oxide is present within the range from 1.0 to 10, preferably 4.0 to 8.0, percent by weight.

The foregoing ranges of tin and antimony oxides are further qualified by the proviso that they be present, respectively, in the range, on a mole ratio basis, of 95:5 to 85:15, especially 90:10. In this fashion, there is obtained the desired doping effect of the antimony on the tin oxide without the presence of an excess separate phase of antimony oxide.

The third component of the mixed coating is "at least one platinum group metal oxide," by which term it is intended to include the oxides of platinum, palladium, ruthenium, iridium, rhodium, and osmium, especially those of ruthenium and iridium. These platinum group metal oxides are present for the most part in their most

highly oxidized state and within the range of from 1.0 to 50, especially 20 to 40, percent by weight. An especially preferred anode is one the coating of which contains a combination of  $\text{RuO}_2$  and  $\text{IrO}_2$ .

The final component is a valve metal oxide selected from the group consisting of titanium and tantalum oxides. Whereas the titanium is present in the form of  $\text{TiO}_2$  and is essentially crystalline (rutile) in nature, when tantalum is employed, a generally amorphous tantalum oxide results. Therefore, although it is expressed as  $\text{Ta}_2\text{O}_5$ , it is understood that mixtures of tantalum oxides may in fact be present. In general,  $\text{Ta}_2\text{O}_5$  is preferred. The amounts of a valve metal oxide employed are generally within the range of from 0.5 to 30 percent by weight, especially 15 to 25 percent.

Thus, a preferred electrode comprises an expanded titanium metal substrate bearing a coating containing about 47 percent  $\text{SnO}_2$ , 5.0 percent  $\text{Sb}_2\text{O}_3$ , 23.5 percent  $\text{RuO}_2$ , 4.5 percent  $\text{IrO}_2$ , and 20 percent  $\text{Ta}_2\text{O}_5$ .

While many of the variety of methods known for producing mixed metal oxide coatings may be employed, the preferred method of preparing the multicomponent coating composition on the titanium substrate is by deposition from a solution of the appropriate thermally decomposable salts. For example, it is desirable to paint or brush an acidified alcoholic solution of said salts onto the substrate, followed by drying at 100°–140° C for from 3 to 10, especially 5, minutes and finally by baking in an oxidizing atmosphere, e.g., air, at 450° to 520° C, especially 500° C, for from 5 to 10, especially about 7, minutes. This procedure may then be repeated any number of times until the desired coating thickness is obtained, for example, 6 to 10 coats. The preferred solvents for the thermally decomposable salts are the lower alkanols such as ethanol, propanol, amyl alcohol, and especially n-butyl alcohol, although other solvents including water may be employed. To these solvents there is generally added from 0 to 50 percent by volume of an acid, such as hydrochloric

sition is incomplete, small amounts of salts may remain without detrimental effect in the coating, for example, small amounts of chloride in the primarily oxide coating.

In order that those skilled in the art may more readily understand the present invention and certain preferred embodiments by which it may be carried into effect, the following specific example is afforded.

#### EXAMPLE

Four anodes were prepared from the following solutions:

Anode 1 — 50 ml n-butanol, 12.5 g  $\text{SnCl}_4 \cdot 5\text{H}_2\text{O}$ , 0.91 g  $\text{SbCl}_3$ , and 1.1 g  $\text{RuCl}_3 \cdot x\text{H}_2\text{O}$  (38% Ru).

Anode 2 — 45 ml ethanol, 5.0 g orthobutyl titanate, 1.1 g  $\text{SbCl}_3$ , 15.1 g  $\text{SnCl}_4 \cdot 5\text{H}_2\text{O}$ , and 7.6 g  $\text{RuCl}_3 \cdot x\text{H}_2\text{O}$  (38% Ru).

Anode 3 — 50 ml n-butanol, 12.5 g  $\text{SnCl}_4 \cdot 5\text{H}_2\text{O}$ , 0.91 g  $\text{SbCl}_3$ , 7.0 g orthobutyl titanate, and 1.1 g  $\text{RuCl}_3 \cdot x\text{H}_2\text{O}$  (38% Ru).

Anode 4 — 45 ml ethanol, 4.5 g  $\text{TaCl}_5$ , 1.1 g  $\text{SbCl}_3$ , 15.1 g  $\text{SnCl}_4 \cdot 5\text{H}_2\text{O}$ , and 7.6 g  $\text{RuCl}_3 \cdot x\text{H}_2\text{O}$  (38% Ru).

Each anode is prepared by applying six coats of the solution by brush to a clean titanium metal mesh with heating in air between each coat, first at 110° C for 3 minutes followed by 7 minutes at 500° C.

These are employed as anodes in a horizontal mercury cell spaced 0.14 inch above and parallel to a mercury cathode flowing at a rate of 450 ml/minute. The electrolyte is a 310 g/l brine solution having a pH within the range of 3–6 and a temperature of about 70° C. To establish the wear-rate of the anodes, electrolysis is continued at 6 amperes per square inch for 500 hours, the loss being determined by weight differential. Efficient low voltage operation is achieved throughout the test. Results, together with the composition of each anode coating calculated on an oxide basis, appear in the following table.

TABLE

| Anode | $\text{SnO}_2\%$ | $\text{Sb}_2\text{O}_3\%$ | $\text{RuO}_2\%$ | $\text{TiO}_2\%$ | $\text{Ta}_2\text{O}_5\%$ | Wear-Rate g/ton $\text{Cl}_2$ |
|-------|------------------|---------------------------|------------------|------------------|---------------------------|-------------------------------|
| 1     | 83.8             | 8.1                       | 8.1              | —                | —                         | 0.29                          |
| 2     | 55.4             | 6.4                       | 30.6             | 7.6              | —                         | 0.25                          |
| 3     | 81.9             | 8.9                       | 7.9              | 1.3              | —                         | 0.14                          |
| 4     | 47.4             | 5.2                       | 27.2             | —                | 20.2                      | 0.11                          |

acid. The concentration of the metals in the solution from which the coating composition is to be derived ranges between about 50 to 200 grams per liter. The salts employed are generally any thermally decomposable inorganic or organic salt or organic ester of the metals in question such as the chlorides, nitrates, alkoxides, alkoxy halides, resinate, amines, and the like. Specific and illustrative examples include potassium hexachloroplatinate, hexachloroiridic acid, ruthenium trichloride or tribromide, orthobutyl titanate, antimony trichloride or pentachloride, and stannic chloride or dibutyl tin dichloride.

It will be understood by those skilled in the art that it is possible to use a number of combinations of preformed oxides of the various component metals and salts of the remaining materials, although it is generally believed that preformed valve metal oxides should not be employed nor should separately preformed tin and antimony oxides be used. Further, if thermal decompo-

50 From the table, it is evident that Anode 1, without the added valve metal oxide, exhibits the highest wear-rate. When tantalum is employed (Anode 4) or using relatively small amounts of titanium (Anode 3), the best results are obtained.

We claim:

55 1. In a process for the electrolysis of brine in a cell with a flowing mercury cathode, the improvement that consists essentially of employing as the anode a titanium substrate bearing on at least a portion of the surface thereof a mixed oxide coating of from 30 to 90 percent by weight  $\text{SnO}_2$ , from 1.0 to 10 percent antimony oxide, calculated as  $\text{Sb}_2\text{O}_3$ , from 1.0 to 50 percent of at least one platinum group metal oxide, and from 0.5 to 30 percent of a valve metal oxide selected from a group consisting of titanium and tantalum oxides, with the proviso that the mole ratio of tin to antimony oxides is between 85:15 and 95:5, and applying current to said anode at a rate of at least 6 amperes per

square inch.

2. An improvement as in claim 1 wherein the anode current density is between 6.0 and 10.0 amperes per square inch.

3. The improvement of claim 1 wherein the platinum group metal oxide is a mixture of RuO<sub>2</sub> and IrO<sub>2</sub>.

4. The improvement of claim 1 wherein the valve

metal oxide is Ta<sub>2</sub>O<sub>5</sub> and is present within the range of 15 to 25 percent.

5. The improvement of claim 1 wherein the coating contains from 30 to 50 percent SnO<sub>2</sub>, 4 to 8 percent antimony oxide, 20 to 40 percent of at least one platinum metal oxide, and 15 to 25 percent Ta<sub>2</sub>O<sub>5</sub>.

\* \* \* \* \*

10

15

20

25

30

35

40

45

50

55

60

65